# EUROPEAN PATENT SPECIFICATION

(11) **EP 2 492 032 B1**
(45) Date of publication and mention of the grant of the patent: **22.10.2014**
(21) Application number: 09848545.1
(22) Date of filing: 17.08.2009
(51) Int. Cl.: B22F 3/26, H01H 33/66, H01H 1/02, C22C 9/00

(54) **METHOD FOR MANUFACTURING A COPPER-BASED COMPOSITE MATERIAL FOR ELECTRICAL CONTACTS**
VERFAHREN ZUR HERSTELLUNG EINES VERBUNDSTOFFES AUF KUPFERBASIS FÜR ELEKTRISCHE KONTAKTE
PROCÉDÉ DE PRODUCTION D UN MATÉRIAU COMPOSITE À BASE DE CUIVRE POUR CONTACTS ÉLECTRIQUES

(43) Date of publication of application: 29.08.2012
(73) Proprietor: Smirnov, Yuriy Iosifovitch, Kiev 02098 (UA)
(72) Inventor: SKOROKHOD, Valeriy Vladimirovitch, Kiev 03150 (UA); CHERNYSHOV, Sergey Ivanovitch, Kharkov 61166 (UA); BARABASH, Vyacheslav Andreevitch, Kiev 03142 (UA); RUPCHEV, Vladimir L'vovitch, Kiev 03118 (UA)
(74) Representative: Benatov, Emil Gabriel
(86) International application number: PCT/UA2009/000042
(87) International publication number: WO 2011/021990

(56) References cited:
- EP-A2- 0 426 490
- WO-A1-90/15424
- JP-A- 63 096 204
- RU-C1- 2 063 086
- US-A- 4 032 301
- US-A- 4 190 753
- US-A- 5 241 745

## Description

The invention relates to powder metallurgy, in particular to methods of manufacturing sintered materials based on copper for electrical contacts used in low voltage and high voltage electrical devices switching circuits, preferably AC circuits with current up to 630 A. In details, the invention relates to method for manufacturing a copper-based composite material for electrical contacts.

In terms of technical essence, the closest analog is a method of manufacturing a copper-based composite material for electrical contacts, comprising preparation of a powder mixture of at least two powder components - conductive and heat resistant components, pressing powder mixture and obtaining a blank, which is sintered to obtain a copper-based composite material for electrical contacts [RF Patent N2 2063086, IPC 6 NH01H33/66, Publ. 1996.06.27].

The disadvantage of the described method is the long duration of the process and, consequently, the high cost of the resulting material for electrical contacts. The long duration of the process is due to the need to perform multiple loadings and unloadings of a vacuum chamber to carry out separate manufacturing operations. In addition, the quality of the produced material is insufficient, in particular, for making contacts of vacuum circuit breakers switching AC circuits with currents even below 400 A due to the impossibility to achieve the required degree of impregnation of the powder mixture of conductive and heat-resistant materials with copper.

The goal of the proposed invention is to provide such method of manufacturing a copper-based composite material for electrical contacts, which would reduce the cost of manufacturing a copper-based composite material for electrical contacts by way of reducing the number of loadings and unloadings of a vacuum chamber to perform three separate technological operations with one vacuum chamber loading, i.e. heating blanks in inert gas or hydrogen atmosphere to a temperature of alloying of interphase border of chromium-copper powder components by a surface-active agent, impregnation of a blank made of copper and chromium powder mixture with alloying components to produce copper layer over blank made of copper and chromium powder mixture, cooling the obtained blank and annealing the blank.

This goals is achieved by the proposed method, which, like the known method of manufacturing a copper-based composite material for electrical contacts, comprises preparation of a powder mixture of at least two powder components - conductive and heat resistant components, pressing powder mixture and obtaining a workpiece, which is sintered to obtain a copper-based composite material for electrical contacts, and, *according to the invention,* copper and chromium powders are preliminarily mixed in a high-power mill to obtain a fine homogenized copper and chromium powder mixture, the obtained powders are pressed to produce two compression-molded briquettes: one of copper and chromium powder mixture and another from copper powder, a source of alloying components is arranged between said compression-molded briquettes, the mixture is heated up to a temperature of 700-900°C in a vacuum chamber under vacuum of 10⁻³ - 10⁻⁵Torr and is kept under these conditions 30-60 minutes to remove unwanted impurities and/or admixtures, which is followed by alloying of interphase border of chromium-copper powder components by surface-active agent in inert gas atmosphere or in hydrogen obtained from metal hydride at a temperature of 1085-1150°C with simultaneous impregnation of compression-molded briquettes of copper and chromium powders with alloying components until a copper layer of a thickness of 2.5-5.0 mm is formed above the compression-molded briquette from a mixture of copper and chromium powder, the obtained blank is cooled from impregnation temperature of 1085-1150°C to a temperature of 900-920°C at a rate equal to or exceeding 20°C/min, the cooled blank is annealed at a temperature of 500-700°C for 30-120 minutes, and a blank of copper-based composite material for producing electrical contacts is obtained.

Another feature of the proposed method is that after obtaining two compression-molded briquettes - from a mixture of copper and chromium powders and from copper powder, a source of alloying components is arranged between these briquettes, such source having a form of a grid.

Another feature of the proposed method is that after obtaining two compression-molded briquettes - from a mixture of copper and chromium powders and from copper powder, a source of alloying components is arranged between these briquettes, such source having a form of a film or foil.

Another feature of the proposed method is that after obtaining two compression-molded briquettes - from a mixture of copper and chromium powders and from copper powder, a source of alloying components is arranged between these briquettes, such source having a form of a coating applied onto the surface of one of the compression-molded briquettes.

Another feature of the proposed method is that after obtaining two compression-molded briquettes - from a mixture of copper and chromium powders and from copper powder, a source of alloying components is arranged between these briquettes, such source having a form of a vacuum coating deposited onto the surface of one of the compression-molded briquettes through mask.

Another feature of the proposed method is that alloying of interphase border of chromium-copper powder components is carried out using surface-active agent of the following composition (in wt.%):
carbon-0.10-0.12
silicon - 0.06 - 0.08
manganese - 1.80 - 2.00
chromium -17.0 -18.0
nickel - 8.90 - 9.00
titanium - 0.70 - 0.80
iron - the rest.

Preliminary processing and blending of copper and chromium powders in high-power mill is aimed at the destruction and deformation of the original powder particles, resulting in formation of active surfaces which are capable of "cold welding" and formation of fine homogenized copper and chromium (Cu-Cr) powder mixture. Such mixture does not segregate by density during unloading from the drum, transportation and loading into the mold matrix. During the processing the mixture is activated, which intensifies the subsequent processes of impregnation and liquid-phase sintering.

The authors have experimentally found the optimal operating conditions of heat treatment of copper and chromium powder mixture in a vacuum chamber. These parameters are: the temperature of 700-900°C, vacuum of 10⁻³ - 10⁻⁵ Torr and maintaining under these conditions for 30 - 60 minutes to remove unwanted impurities and/or admixtures. It was found out that under temperatures below 700°C and keeping in a vacuum chamber during less that 30 minutes copper and chromium powder mixture still contains volatile oxides, which have a negative impact on the quality of the obtained product. Heating of the mixture above 900°C triggers evaporation of chromium (at the temperature of 907°C) and copper (at the temperature of 946°C). Vacuum below 10⁻³ Torr is not effective, because there were cases of powders oxidation observed. Vacuum over 10⁻⁵ Torr is not economically justified, because further vacuum increase does not significantly improve the quality of the resulting material. In case of keeping the powders under these conditions for less than 30 minutes, the cases of incomplete removal of unwanted impurities, in particular oxide films, were observed. Increase of dwelling time over 60 minutes is not economically justified, because it does not significantly improve the quality of the resulting material.

Placement of the source of alloying components between obtained compression-molded briquettes of copper powder and copper-chromium powder mixture enables, under further heating of the blanks in an inert gas atmosphere at a temperature of 1085-1150°C and dwelling time of 15-20 minutes, to perform the alloying of interphase border of chromium-copper powder components with surface-active substance with simultaneous impregnation of copper and chromium powder mixture briquette with alloying components to form 2.5 - 5.0 mm thick copper layer over the briquette of copper and chromium powder mixture. This process occurs due to improvement of chromium wetting with copper, which results in more intense impregnation, reducing the number and size of closed pores in the contact material, improvement of thermal-physical properties and reducing the process time. The optimum temperature in a vacuum chamber 1085-1150°C is determined experimentally by the authors. The lower limit of temperature in the vacuum chamber 1085°C corresponds to copper melting point, so it can not be lowered. Increasing the temperature above 1150°C leads to copper evaporation, which reduces the effectiveness of briquette impregnation. The copper layer thickness of 2.5 - 5.0 mm over the briquette of copper and chromium powder mixture is determined by the future operating conditions of the contact pair manufactured from the produced material, i.e. rated current, switching frequency, the nature of the load. The thickness of the copper layer is determined by the concentration of surface-active components, which are intended to improve the wettability of chromium powder by liquid copper and decrease the surface tension of molten copper, i.e. reducing the height of liquid copper meniscus over the surface of the briquette of chromium and copper powder mixture, as well as the copper quantity itself.

The subsequent cooling of the blank from impregnation temperature to the temperature of 900-920°C is performed at a rate equal to or greater than 20 degrees per minute in order to fix the fine structure of chromium-copper and copper and to reduce the likelihood of shrinkage cavities. The authors have experimentally determined that the blank cooling rate below 20 degrees per minute results in increasing grains in the structure of the future blank, which does not allow to obtain high-quality material.

The resulting blank is annealed under these optimal parameters: temperature of 500-700°C, 30 - 120 minutes. Because only with these parameters the blank maintains fine structure and tensions in the lattice are decreased. These optimal parameters were found experimentally by the authors. The heating to a temperature below 500°C and during less than 30 minutes adversely affects the quality of the finished product, since there were cases of incomplete relaxation of stresses in the blank. Heating at the temperature over 700°C during more than 120 minutes is not justified economically, because it practically has no effect on the quality of the finished product.

Source of alloying components can be made in the form of foil, grid or vacuum coating. Its design is determined by the technological possibilities of the material manufacturer. The authors believe, the most promising structure is a vacuum coating deposited on the flat surface of one of the blanks through a mask, because it provides the desired composition and necessary amount of alloying components. The simplest structure is a foil. In this case it is sufficient to obtain the melt of necessary composition or select a ready metallic material or alloy in the form of an ingot of the necessary composition and with required amount of alloying components, heat it and roll it between the rollers to obtain a foil of the desired thickness.

Surface-active agents are used in an amount of 1-3 wt.% of the total weight of the contact material to improve wettability and activation of the sintering and impregnation process.

The composition and quantity of the alloying components for alloying the interphase border of chromium-copper powder components are selected experimentally based on conditions to improve the wetting of interphase border by copper melt and to reduce the surface tension of molten copper in the mixture of chromium-copper powders. Such substances for chrome-copper - copper melts may be substances based on silicon, manganese, nickel, and are selected experimentally based on the technological possibilities of the material manufacturer and the intended working conditions of the contact material.

As an example, the authors have used for alloying of interphase border of chromium-copper powder components a source of alloying components of the following composition (in wt.%):
carbon-0.10-0.12
silicon - 0.06 - 0.08
manganese - 1.80 - 2.00
chromium - 17.0 - 18.0
nickel - 8.90 - 9.00
titanium - 0.70 - 0.80
iron - the rest.

Fig. 1 illustrates a blank of electric contact Cu-Cr material with a copper sublayer, obtained by the proposed method.

Example. The copper-based composite material for electrical contacts was produced. The following materials were used: electrolytic copper powder according to GOST 4960-75, PMS-1 grade with a copper content of 99.72%, and chromium powder of PH-1M grade, a certificate # 22-03 of 02.10.2008.

The operations of mixing and grinding of copper and chromium powders was carried out in a high power mill. A planetary mill, attritor, ball mill etc. may be used as a device for mixing and grinding powders. Blend modes (operating tools rotation speed, mixing time, balls mass to material mass ratio, etc.) were selected experimentally. The balls impact on the components of the treated powder material exceeds the ultimate compressive strength and shear of plastic copper and solid chromium. The amount of copper (Cu) powder introduced into chromium (Cr) during the mixture preparation was 10-40 wt.%, depending on the Cr content in the composition of the contact material, with increasing of Cr content in the Cu-Cr composition from 45 to 70 wt.%, the amount of copper in Cu-Cr mixture was decreased from 40 to 10 wt.%, respectively. The processing and blending of copper and chromium powders in high-power mill resulted in destruction and deformation of the original powder particles, which leaded to formation of active surfaces which were capable of "cold welding" of microgranules that caused formation of fine homogenized copper and chromium (Cu-Cr) powder mixture. Such mixture did not segregate by density during unloading from the drum, transportation and loading into the mold matrix. During the processing the mixture was activated, which intensified the subsequent processes of impregnation and liquid-phase sintering.

To obtain the briquettes of required shape and size, the Cu-Cr powder mixture was subjected to pressing in molds. Cu concentration in Cu-Cr mixture and the residual porosity of the compressed briquette are the main parameters determining the amount of Cr in the manufactured composite material after the obtaining a blank impregnated with copper melt. The minimum Cr amount in Cu-Cr composite material manufactured according to the principle of forming rigid Cr structure impregnated with Cu is about 45 wt.% according to specific weights of Cr - 7.15 g/cm³ and Cu - 8.93 g/cm³.

The maximum amount of Cr in the composite material is determined by the possibility to form a raw briquette with a minimum amount of Cu in Cu-Cr mixture and minimum porosity of compression-molded briquette without cracking and is about 70 wt.%. Cu-Cr blanks were pressed using the pressure from 2 to 8 tons per square cm. Increasing of the compression pressure over 8 tons per square cm results in delamination of the compression-molded blanks. With increasing Cr concentration in the composite material the compression pressure was increased. In order to impregnate the blanks, the briquettes of copper powder (chips) were pressed together with alloying components source. For uniform distribution of surface-active elements at the Cr-Cu interphase border and facilitation of compression, the source of allying components is made in the form of foil, grids of different shape, discrete vacuum coating. Such coating may be applied by known methods, for example, using a process described in the article: - 1997. - No11/12. - P.93-96. (The wear resistance of silicon nitride based ceramic cutting tools with continuous and discrete nitride titanium coatings. Gnesin, G.G., Lyashenko, B.A., Fomenko, S.N. et al. - Powder Metallurgy). A grid or foil of alloying components is placed into the lower mold die and covered with necessary amount of copper powder or chips, and then press the composite blank using the pressure of 1.5-3.0 tons per square cm.

For uniform distribution of surface-active elements at the Cr-Cu interphase border and facilitation of compression, the source of allying components is made in the form of foil, grids of different shape, vacuum coating.

### Heat vacuum treatment:

Connected porous briquette of Cu-Cr powders mixture, Cu powder briquette and a source of alloying components located between the briquettes were subjected to heat vacuum treatment together. Briquettes were placed into container made of a material which does not react with molten Cu and Cr. The copper briquette was placed onto upper surface of the briquette in such a way that grid with surface-active substance was in contact with the surface of Cu-Cr blank. Container was placed into vacuum over chamber. Heat vacuum treatment was performed in a vacuum chamber in vacuum of 10⁻⁵Torr, at 800°C for 60 min to remove adsorbed gases, volatile components from the blanks, to destroy and remove oxide films. After heating and keeping for 60 minutes inert gas or hydrogen produced from the metal hydride was supplied into vacuum chamber through the inlet valve to produce a pressure of 200 Torr and the temperature was raised to 1150°C at a rate of 10-15 degrees per minute.

### Impregnation.

Copper melting and alloying of chromium-copper (Cr-Cu) interphase border with surface-active components, liquid-phase sintering of briquettes and their impregnation with copper occurs in the temperature range of 1085-1150°C in inert gas or hydrogen atmosphere. The blank was kept during 10-20 minutes in this temperature interval. Optimum dwelling time was selected experimentally depending on the blank mass, heat capacity and pressure of the gas atmosphere.

The amount of copper necessary for impregnation of the blank (structure) was calculated on the basis of its residual porosity and the amount of copper required for the formation of a 2.5 - 5 mm thick layer intended to divert heat flow from the working surface of the contact assembly and welding or soldering of the contact to arc-suppression vacuum chamber terminals.

In the example, the source of alloying components is in the form of a grid having the following composition (in wt.%): C-0.12; Si-0.08; Mn-2.0; Cr-18.0; Ni-9.0; Ti-0.8; Fe - up to total of 100.0. The mass of the source of the alloying components is in the range from 1.0 to 3.0 wt.% of the total mass of the contact material. A source of alloying components is used in order to improve the wettability and facilitate the processes of sintering and impregnation.

### Cooling.

In order to obtain the blanks with fine structure, impregnated Cu-Cr blanks were cooled from the impregnation temperature to the crystallization temperature at a rate of 20-28 degrees/min.

To relieve internal stresses, the structure was annealed in inert medium at 650-670°C for 120 minutes.

Thus, the proposed invention has enabled to achieve the goal: to provide such method of manufacturing a copper-based composite material for electrical contacts, with the cost of manufacturing of such electrical contacts lower that the cost of manufacturing contacts made of material obtained according to prototype process due to creation of conditions allowing to reduce the number of loadings and unloadings of a vacuum chamber to perform three separate technological operations with one vacuum chamber loading, i.e. heating blanks in inert gas or hydrogen atmosphere to a temperature of alloying of interphase border of chromium-copper powder components by a surface-active agent, impregnation of a blank made of copper and chromium powder mixture with alloying components to produce copper layer over blank made of copper and chromium powder mixture, cooling the obtained blank and annealing the blank.

The resulting composite material for contacts was tested in contactors operating in power circuits of the rolling stock of Ukrainian railways. The service life of contacts made of the proposed composite contact material was 50-60% longer than the service life of conventional contacts.

## Claims

1. A method of manufacturing a copper-based composite material for electrical contacts comprising preparation of a powder mixture of at least two powder components - conductive and heat resistant components, pressing powder mixture and obtaining a blank, which is sintered to obtain a copper-based composite material for electrical contacts, ***characterized in that*** copper and chromium powders are preliminarily mixed in a high-power mill to obtain a fine homogenized copper and chromium powder mixture, the obtained powders are pressed to produce two compression-molded briquettes: one of copper and chromium powder mixture and another from copper powder, a source of alloying components is arranged between said compression-molded briquettes, the mixture is heated up to a temperature of 700-900°C in a vacuum chamber under vacuum of 10⁻³ - 10⁻⁵ Torr and is kept under these conditions for 30-60 minutes to remove unwanted impurities and/or admixtures, which is followed by alloying of interphase border of chromium-copper powder components by surface-active agent in inert gas atmosphere or in hydrogen obtained from metal hydride at a temperature of 1085-1150°C with simultaneous impregnation of compression-molded briquettes of copper and chromium powders with alloying components until a copper layer of a thickness of 2.5-5.0 mm is formed above the compression-molded briquette from a mixture of copper and chromium powder, the obtained blank is cooled from impregnation temperature of 1085-1150°C to a temperature of 900-920°C at a rate equal to or exceeding 20°C/min, the cooled blank is annealed at a temperature of 500-700°C for 30-120 minutes, and a blank of copper-based composite material for producing electrical contacts is obtained.

2. A method according to claim 1, ***characterized in that*** after obtaining two compression-molded briquettes - from a mixture of copper and chromium powders and from copper powder, a source of alloying components is arranged between these briquettes, such source having a form of a grid.

3. A method according to claim 1, ***characterized in that*** after obtaining two compression-molded briquettes - from a mixture of copper and chromium powders and from copper powder, a source of alloying components is arranged between these briquettes, such source having a form of a foil.

4. A method according to claim 1, ***characterized in that*** after obtaining two compression-molded briquettes - from a mixture of copper and chromium powders and from copper powder, a source of alloying components is arranged between these briquettes, such source having a form of a coating applied onto the surface of one of the compression-molded briquettes.

5. A method according to claim 1, ***characterized in that*** after obtaining two compression-molded briquettes - from a mixture of copper and chromium powders and from copper powder, a source of alloying components is arranged between these briquettes, such source having a form of a vacuum coating deposited onto the surface of one of the compression-molded briquettes through mask.

6. A method according to claim 1, ***characterized in that*** alloying of interphase border of chromium-copper powder components is carried out using surface-active agent of the following composition (in wt.%):
carbon-0.10-0.12
silicon - 0.06 - 0.08
manganese - 1.80 - 2.00
chromium -17.0 -18.0
nickel - 8.90 - 9.00
titanium - 0.70 - 0.80
iron - the rest.

## Patentansprüche

1. Verfahren zur Herstellung eines Verbundwerkstoffs auf Kupferbasis für elektrische Kontakte, einschließlich die Bereitstellung einer Pulvermischung aus mindestens zwei Pulverkomponenten - leitenden und wärmebeständigen Komponenten, das Zusammenpressen der Pulvermischung und das Erhalten eines Rohlings, der gesintert wird, um einen Verbundwerkstoff auf Kupferbasis für elektrische Kontakte zu erhalten, **dadurch gekennzeichnet, dass** Kupfer-und Chrompulver vorläufig in einer Hochleistungsmühle gemischt werden, um ein fein homogenisiertes Kupfer- und Chrom-Pulvergemisch zu erhalten; die erhaltenen Pulver gepresst werden, um zwei pressgeformte Briketts herzustellen: das eine aus Kupfer- und Chrom-Pulvermischung und das andere aus Kupferpulver, zwischen der Pressformbriketts ist eine Quelle von Legierungskomponenten angeordnet, das Gemisch wird bis zu einer Temperatur von 700-900 °C in einer Vakuumkammer bei einem Vakuum von 10⁻³ - 10⁻⁵ Torr erhitzt und unter diesen Bedingungen für 30-60 Minuten gehalten, um unerwünschte Verunreinigungen und/oder Zusätzen zu entfernen, gefolgt vom Legieren der Zwischenphasengrenze zwischen den Komponenten des Chrom-Kupfer-Pulvers bei einem oberflächenaktiven Mittel in einer inerten Gasatmosphäre oder in Wasserstoff, gewonnen aus Metallhydrid bei einer Temperatur von 1085-1150 °C bei gleichzeitiger Imprägnierung der Pressformbriketts aus Kupfer- und Chrompulver mit Legierungsbestandteilen, bis eine Kupferschicht mit einer Stärke von 2,5-5,0 mm über das Pressformbrikett aus Mischung von Kupfer- und Chrompulver gebildet wird; der erhaltene Rohling aus der Imprägnierungstemperatur von 1085-1150 °C auf eine Temperatur von 900 bis 920 °C mit einer Geschwindigkeit von gleich oder über 20 °C/min gekühlt wird, der gekühlte Rohling bei einer Temperatur von 500-700 °C für 30-120 Minuten geglüht wird, und ein Rohling aus Verbundwerkstoff auf Kupferbasis zur Herstellung elektrischer Kontakte erreicht wird.

2. Verfahren nach Anspruch 1, **dadurch gekennzeichnet, dass** nach dem Erhalten von zwei Pressformbriketts - aus einer Mischung aus Kupfer- und Chrompulver und aus Kupferpulver - eine Quelle von Legierungskomponenten zwischen die Briketts angeordnet wird, wie Quelle mit einer Gitterform.

3. Verfahren nach Anspruch 1, **dadurch gekennzeichnet, dass** nach dem Erhalten von zwei Pressformbriketts - aus einer Mischung aus Kupfer- und Chrompulver und aus Kupferpulver - eine Quelle von Legierungskomponenten zwischen die Briketts angeordnet wird, wie Quelle mit der Form einer Folie.

4. Verfahren nach Anspruch 1, **dadurch gekennzeichnet, dass** nach dem Erhalten von zwei Pressformbriketts - aus einer Mischung aus Kupfer- und Chrompulver und aus Kupferpulver - eine Quelle von Legierungskomponenten zwischen die Briketts angeordnet wird, wie Quelle mit der Form einer Beschichtung, die auf die Oberfläche einer der Pressformbriketts aufgebracht ist.

5. Verfahren nach Anspruch 1, **dadurch gekennzeichnet, dass** nach dem Erhalten von zwei Pressformbriketts - aus einer Mischung aus Kupfer- und Chrompulver und aus Kupferpulver - eine Quelle von Legierungskomponenten zwischen die Briketts angeordnet wird, wie Quelle mit der Form einer Vakuumbeschichtung, die durch die Maske auf die Oberfläche eines der Pressformbriketts abgeschieden ist.

6. Verfahren nach Anspruch 1, **dadurch gekennzeichnet, dass** das Legieren der Zwischenphasengrenze zwischen den Komponenten des Chrom-Kupfer-Pulvers unter Verwendung von oberflächenaktiven Mittels mit der folgenden Zusammensetzung (in. Gew.%) durchgeführt wird:
Kohlenstoff - 0,10 bis 0,12
Silizium - 0,06-0,08
Mangan - 1,80-2,00
Chrom -17,0 -18,0
Nickel - 8,90 - 9,00
Titan - 0,70-0,80
Eisen - der Rest.

## Revendications

1. Procédé de fabrication d'un matériau composite à base de cuivre destiné pour des contacts électriques comprenant la préparation d'un mélange en poudre constitué d'aux moins deux components en poudre - conductible et résistant à la chaleur, la compression du mélange en poudre et l'obtention d'une ébauche qui est soumise au frittage pour obtenir un matériau composite à base de cuivre destiné pour des contacts électriques, ***caractérisé en ce que*** les poudres du cuivre et du chrome sont préalablement mélangées dans un broyeur a haute puissance pour obtenir un mélange de cuivre et de chrome en poudre de homogénéité fine, les poudres obtenus sont compressés pour donner deux briquettes moulées par compression : l'une à partir du mélange de cuivre et de chrome en poudre et l'autre à partir du cuivre en poudre, une source de composants d'alliage est placée entre les briquettes moulées par compression, le mélange est chauffé jusqu'à une température de 700-900°C dans une chambre à vide sous 10⁻³ - 10⁻⁵ Torr et est maintenu dans ces conditions pendant 30 à 60 minutes pour éliminer les impuretés et/ou les adjuvants non désirés, puis suit alliage de l'interphase de frontière des composants de cuivre et de chrome en poudre à l'aide d'un agent tensio-actif dans une atmosphère de gaz inerte ou de l'hydrogène obtenu à partir d'un hydrure de métal à une température de 1085-1150°C et avec une imprégnation simultanée des briquettes moulées par compression de cuivre et de chrome en poudre avec les composants d'alliage jusqu'à ce qu'une couche de cuivre d'épaisseur de 2,5-5,0 mm est formée sur les briquettes moulées par compression à partir d'un mélange de cuivre et de chrome en poudre, l'ébauche obtenue est refroidi à partir de la température de l'imprégnation de 1085-1150°C jusqu'à une température de 900-920°C à une vitesse égale ou supérieure à 20°C/min, l'ébauche refroidie est recuite à une température de 500-700°C pendant 30 à 120 minutes, et est obtenue une ébauche de matériau composite à base de cuivre pour la production des contacts électriques.

2. Procède selon la revendication 1, ***caractérisé en ce qu'**après* l'obtention des deux briquettes moulées par compression - à partir d'un mélange de cuivre et de chrome en poudre et à partir de cuivre en poudre, une source de composants d'alliage est disposée entre ces briquettes, la source étant en forme d'une grille.

3. Procède selon la revendication 1, ***caractérisé en ce qu'**après* l'obtention des deux briquettes moulées par compression - à partir d'un mélange de cuivre et de chrome en poudre et à partir de cuivre en poudre, une source de composants d'alliage est disposée entre ces briquettes, la source étant en forme d'une feuille.

4. Procède selon la revendication 1, ***caractérisé en ce qu'**après* l'obtention des deux briquettes moulées par compression - à partir d'un mélange de cuivre et de chrome en poudre et à partir de cuivre en poudre, une source de composants d'alliage est disposée entre ces briquettes, la source étant en forme d'un revêtement appliqué sur la surface de l'une des briquettes moulées par compression.

5. Procède selon la revendication 1, ***caractérisé en ce qu'**après* l'obtention des deux briquettes moulées par compression - à partir d'un mélange de cuivre et de chrome en poudre et à partir de cuivre en poudre, une source de composants d'alliage est disposée entre ces briquettes, la source étant en forme d'un revêtement à vide appliqué sur la surface de l'une des briquettes moulées par compression à travers un masque.

6. Procède selon la revendication 1, ***caractérisé en ce que*** l'alliage de l'interphase de frontière des composants chrome-cuivre est effectué en utilisant des agents tensio-actifs de la composition suivante (% en poids) :
carbone - 0,10 à 0,12
silicium - 0,06 à 0,08
manganèse - 1,80 à 2,00
chrome -17,0 -18,0
nickel - 8,90 à 9,00
titane - 0,70 à 0,80
fer - le reste.
